

Sept. 15, 1959

F. H. HORN

2,904,512

GROWTH OF UNIFORM COMPOSITION SEMICONDUCTOR CRYSTALS

Filed July 2, 1956



Inventor:  
Fordyce Hubbard Horn,  
by Richard R. Brainerd  
His Attorney.

1

2,904,512

## GROWTH OF UNIFORM COMPOSITION SEMICONDUCTOR CRYSTALS

Fordyce Hubbard Horn, Schenectady, N.Y., assignor to General Electric Company, a corporation of New York

Application July 2, 1956, Serial No. 595,503

7 Claims. (Cl. 252—62.3)

The present invention relates to methods for growing semiconductor single crystals. More particularly, the invention relates to methods for growing semiconductor single crystals having therein a substantially constant concentration of impurities.

Semiconductor materials such as germanium and silicon are of great importance, particularly in the construction of asymmetrically conductive devices such as rectifiers and transistors. Such devices require monocrystalline semiconductor bodies with predictable and substantially constant impurity distributions. Generally, the crystalline bodies from which such semiconductor devices are formed, are prepared by subjecting a semiconductor monocrystalline body having a constant impurity concentration to one or more physical operations such as alloying or melting and refreezing. Accordingly, there is a great need in the electronics industry for methods of growing semiconductor single crystals having uniform impurity distributions.

Presently available methods for preparing transistor grade semiconductor materials are not completely suitable for preparing unconstrained single crystals of semiconductor materials having a constant concentration of impurities therein immediately suitable for transistor uses. Thus for example the Czochralski seed crystal withdrawal method, which is used to produce high purity semiconductor single crystals, is incapable of producing single crystal having constant impurity concentration. This is so because the method involves growing a crystal from a completely molten bath of semiconductor material impregnated with a given concentration of significant impurities. Since the segregation coefficients of the electrically significant impurities in silicon and germanium are generally markedly less than unity, the concentration of such impurities in the melt from which a crystal is grown progressively increases as a crystal is grown therefrom, resulting in a progressively increasing concentration of these impurities in the grown crystal.

The zone melting method of forming semiconductor bodies having therein uniformly distributed impurities is not well adapted to the production of single crystals. It is extremely difficult to form a single crystal of a semiconductor material in a crucible as is done in zone-melting. Even if such difficulties are overcome and a single crystal is grown, the growth of the crystal within the confines of a crucible or boat results in the introduction of strains in the crystal due to its growth under constraint. Such strains are intolerable, and must be removed by annealing, which requires further heat treatment of the crystal for many hours or even days.

Accordingly, one object of the invention is to provide a method for the unconstrained growth of single crystals of semiconductor materials having therein a constant concentration of electrically significant impurities.

Another object of the invention is to provide a method for growing single crystals of semiconductor materials

2

having therein a constant concentration of electrically significant impurities and which require no further treatment to render them suitable for use in transistor devices.

In accord with my invention, I prepare unconstrained 5 single crystals of semiconductor materials having therein a uniform distribution of electrically significant impurities having a segregation coefficient less than unity by growing a single crystal by seed crystal withdrawal from a substantially constant volume molten zone of a 10 semiconductor material maintained within a crucible. As the single crystal is grown, the molten zone is constantly replenished by continuously melting solidified semiconductor material within the crucible. Crystals grown by this method have a uniform distribution of impurities 15 therein, are unconstrained, and are ready for immediate use in the preparation of semiconductor devices.

The novel features believed characteristic of the invention are set forth in the appended claims. The invention itself together with further objects and advantages there- 20 of may best be understood by reference to the attached drawing in which the sole figure is a cross-sectional view of an apparatus suitable for use in the practice of the invention.

The illustrated apparatus includes a refractory furnace 25 envelope 1 having a closed base 2 and an open flanged upper end 3. Envelope 1 is preferably cylindrical in shape and is much longer than its diameter. In the upper portion of the cylinder of furnace envelope 1 there is located an input feeder tube 4 disposed at an acute angle to the 30 axis of envelope 1 and closed by a spring biased closure member 5 having a central aperture 6 therein, closed by a ball check valve 7. Within cylindrical envelope 1 is located a cylindrical crucible 8 having a depth dimension at least 1½ times its diameter which is guided to a central 35 position by a sleeve member 9 and a centering spring 10. Crucible 8 is supported upon a suitable annular, outwardly flanged support member 11 conveniently packed with a mass of quartz wool 12. Furnace envelope 1, spacer 9, crucible 8 and support member 11 are conveniently fabricated from quartz.

The upper, open end of envelope 1 is fastened to a 40 closure plate 13 which is spaced from a pair of supported plates 14 and 15 by means of vertical rods 16 and 16'. Plates 13, 14 and 15 comprise a part of the apparatus for regulating the movement of movable parts of the apparatus as will be more fully described hereinafter. Closure plate 13 has an aperture 17 therein for the passage 45 of a crystal drawing mandrel 18 therethrough. An airtight seal 19 maintains a closed atmosphere within furnace envelope 1 and allows for the passage of mandrel 18 therethrough. Mandrel 18 is fastened by coupling 20 to a threaded shaft 21 which passes through supporting plate 14 and is connected through a suitable step-down gear mechanism 22 to gear ratio control box 23. Control box 23 serves as a distributor for driving energy 50 supplied by electric motor 24 and contains suitable clutches for the drive-shafts operated therefrom so that they may be turned manually when desired. A second drive shaft 25 drives coil holder 26 from gear control box 23 and raises and lowers radio frequency inductance heating coils 27 and 28 with respect to crucible 8 within furnace envelope 1. Gear control box 23 adjusts the relative speed 55 ratio of mandrel 18 and drive shaft 25 so that mandrel 18 is raised at a first preselected rate and induction heating coils 27 and 28 are lowered at a second preselected rate.

A mass 29 of semiconductor material, such as germanium or silicon is located in crucible 8. A zone 30 of semiconductor mass 29 is maintained in the molten state and a single crystal 31 of semiconductor material is grown therefrom by seed crystal withdrawal. Ingot 31 is grown upon seed crystal 32 which is maintained in chuck 33

attached to mandrel 18. Radio frequency energy for heating semiconductor 29 in crucible 8 is supplied to RF induction coils 27 and 28, which are electrically in series, by means of conductors 34 and 35 which are connected to a radio frequency oscillator. During the entire operation a protective gas, as for example argon, is caused to flow into envelope 1 through inlet conduit 37 and escapes through aperture 38 in the base of envelope 1.

In practicing the invention a mass 29 of semiconductor material having a known impurity content is placed within crucible 8. Conveniently semiconductor mass 29 may be prepared by zone melting and may have the characteristics of intrinsic semiconductor, with a resistivity of in excess of 30 ohm centimeters in the case of germanium and 100 ohm centimeters in the case of silicon. Radio frequency power is supplied through conductors 34 and 35 to induction heating coils 27 and 28 to completely melt the charge of semiconductor material within crucible 8. Conveniently mass 29 may be preheated by a resistance coil (not shown) to make the semiconductor more conductive and more receptive to induction heating. If the material being melted is germanium, the temperature must be raised above 941° C., and if the semiconductor material utilized is silicon, the temperature must be raised above 1420° C.

When the entire mass 29 of semiconductor material in crucible 8 has been melted, the power supplied to induction coils 27 and 28 is abruptly lowered so that the entire crucible full of semiconductor material solidifies nondirectionally but is maintained above a temperature at which the semiconductor remains plastic. It is an important feature in the practice of the invention that once the semiconductor mass 29 in crucible 8 has been melted, and allowed to refreeze, it is maintained above a temperature at which the semiconductor remains plastic. This is necessary to prevent expansion upon complete cooling, and a consequent fracture of the crucible. Thus, for example, if the material utilized is germanium, the refrozen material within the crucible is maintained at a temperature in excess of 600°. If the material is silicon, it is maintained at a temperature in excess of 1000° C. As soon as semiconductor material 29 has refrozen, coil holder 26 is manually adjusted so that heater coil 27 is adjacent the upper surface of the material within the crucible. The power to induction heating coils 27 and 28 is then increased until a molten zone 30 forms at the top of semiconductor mass 29. A molten zone forms only at the top of the crucible because the number of turns on induction coil 27 is much greater than the number of turns for coil 28, and the heat energy supplied to the upper end of the frozen material within crucible 8 is sufficient to melt the semiconductor contained therein, while the remainder of the frozen ingot remains solid. The thickness of molten zone 30 may be adjusted by changing the number of turns upon radio frequency coil 29, or by increasing or decreasing the power thereto. The thickness of zone 31 is conveniently adjusted to from approximately 1/2 to 3/4 of the diameter of the crucible used.

If semiconductor material 29 is high-purity or intrinsic semiconductor, molten layer 30 is then inoculated with the concentration of a significant activator impurity sufficient to supply to crystalline ingot 32 grown in equilibrium therewith the desired concentration of the impurity. This amount for small values of K may be calculated from the simplified relationship

$$C = KC_i \quad (1)$$

where

C is the concentration of the impurity within the ingot to be grown

K is the segregation coefficient of the impurity in the semiconductor utilized and

C<sub>i</sub> is the concentration of the impurity in the molten zone

Mandrel 18 is next manually lowered until seed crystal 32 is in contact with the surface of molten zone 30. The seed crystal is left in this position until it is observed to fuse with the molten zone. Mandrel 18 and drive shaft 25 are then connected directly to gear ratio box 23 as for example by clutches therein, and driving power is then supplied to gear ratio control 23 to cause mandrel 18 to slowly rotate and rise. The speed of rotation of mandrel 18 and hence seed crystal 32 is not critical, since rotation is not necessary. Conveniently, the mandrel may be rotated at a speed of 100 revolutions per minute. The threads upon threaded shaft 21 mesh with an internally threaded coupling 36 on plate 14 and cause mandrel 18 and seed crystal 32 to slowly rise. The rate of "pulling" or the rate of rise of seed crystal 31 may be any rate less than 6 inches per hour and is conveniently chosen in accord with the time cycle desired. As mandrel 18, and consequently seed crystal 32 rises, a monocrystalline ingot 31 of semiconductor material impregnated with a concentration C of the chosen significant impurity element is grown from molten zone 30.

As crystal 31 is grown the amount of semiconductor material within molten zone 30 would be decreased if no compensation were made for the material lost to crystal 32. Therefore, by means of gear ratio box 23, drive shaft 25 which is clutched to operate automatically at the same time mandrel 18 is so clutched is geared to rotate and to lower induction heating coils 27 and 28 at a speed which is related to the speed at which seed crystal 32 is withdrawn by a ratio approximately inversely proportional to the ratio of the cross-sectional area of crucible 8 and the cross-sectional area of monocrystalline ingot 31.

More particularly the ratio of these rates is governed by the relationship

$$\frac{P}{L} = \frac{D^2}{d^2} - 1 \quad (2)$$

where

P = the rate of crystal withdrawal

L = the rate at which the molten zone is lowered

D = the diameter of the crucible

d = the diameter of the growing crystal

It will be appreciated that in order to grow unconstrained single crystals in accord with the invention d must always be less than D.

By virtue of this regulation, molten zone 30 is continually maintained at a substantially constant volume. Since the vast majority of the significant activator impurities added to molten zone 30 are segregated out of growing crystal 31, the concentration of significant activator impurity material within molten zone 30 remains substantially constant. This is particularly true for segregation coefficients of less than 0.05. As is well known to the art, the segregation coefficient of an impurity in a semiconductor grown from a liquid melt with which it is in equilibrium is defined as the ratio of the concentration of the impurity in the growing crystal to the concentration of the impurity within the melt. The method of the invention is suited for growing semiconductor crystals having therein a constant concentration of significant activator impurities having segregation coefficients less than unity. It is, however, preferably practiced with impurities having segregation coefficients less than 0.05 but greater than 0. Since the volume of molten zone 30 remains substantially constant, and since the concentration of significant activator impurities therein remain substantially constant, the concentration of activator impurities within growing crystal 31 is substantially constant until the ingot is grown to full size, and only a small amount of residual semiconductor remains in the bottom of crucible 8.

In this respect it should be noted that the diameter of bottom flange 2 on furnace envelope 1 is smaller than the inside diameter of RF coils 27 and 28 thus permitting

the coils to be lowered below the lowest extremity of furnace 1 to grow an ingot from substantially the entire charge of semiconductor within the crucible.

The process of the invention may be practiced with additions of numerous impurities to semiconductors such as germanium or silicon. As used herein, the term "impurity" does not connote an undesirable inclusion within the semiconductor body but connotes an electrically significant inclusion which, because of its presence in small amounts, is responsible for the highly desirable semiconducting properties of semiconductive materials. Such impurities are divided into two principal groups which are electrically significant. These groups are the acceptors of group III of the periodic table which include aluminum, gallium and indium, and the donors of group V of the periodic table which include phosphorus, arsenic and antimony. All of these impurities have segregation coefficients in both germanium and silicon less than unity. A third, but less-known group of electrically significant impurities in germanium and silicon are the elements which introduce deep trapping levels into the semiconductor energy scheme. These materials include iron, nickel, cobalt, manganese, zinc and gold. All of these materials have segregation coefficients in germanium and silicon less than .001 and are, therefore, ideally suited for use in the practice of this invention. The characteristics of these materials in germanium may be found in an article entitled "Scattering of Carriers From Doubly Charged Impurity Sites in Germanium," by W. W. Tyler and H. H. Woodbury, vol. 102, Physical Review, page 647, May 1, 1956, and the references cited therein.

In order to grow semiconductor single crystals having therein a substantially constant concentration of electrically significant impurities in accord with the method of the invention, it is preferable that the segregation coefficient of the selected impurity in the semiconductor material be lower than 0.05. Thus, for example, when indium, having a segregation coefficient of 0.001, arsenic having a segregation coefficient of 0.04 or antimony having a segregation coefficient of 0.003, are added to a molten zone of a germanium melt and the method practiced in accord with the foregoing disclosure, a single crystalline semiconductor ingot may be produced having less than a 10% variation in the concentration of impurities from one end to the other. Such a condition is ideal. However, semiconductor ingots of germanium having an impurity distribution well within the specifications and needs for the production of semiconductor devices such as transistors and rectifiers may be grown in accord with this invention utilizing, as well as the aforementioned impurities, aluminum, gallium and phosphorus all of which have a segregation coefficient in germanium equal to 0.1. While a crystal grown from a germanium melt in accord with the invention having a molten zone inoculated with aluminum, gallium or phosphorus does not have a completely uniform distribution of these impurities from one end to the other, the variation is not great enough to detract from the usefulness of the germanium as a source of material for the production of semiconductor devices.

In silicon, indium having a segregation coefficient of 0.0003, gallium having a segregation coefficient of 0.004, aluminum having a segregation coefficient of 0.002, and antimony having a segregation coefficient of 0.02 may all be used in the practice of the invention for the production of silicon crystals having a substantially constant concentration of these impurities along a single crystal ingot. With arsenic or phosphorus in silicon the situation is somewhat different. Both of these materials have a segregation coefficient in silicon equal to 0.3. Because of this rather high segregation coefficient, if the volume of molten zone 30 is maintained constant as crystal 31 is grown therefrom, the concentration of these impurities of the grown crystal falls substantially, as the ingot is grown. Such a condition, however, may be compensated

70  
75

for, in the case of these two impurities, by a very simple modification. This may be accomplished by the simple expedient of progressively decreasing the thickness of molten zone 30 as ingot 31 is grown therefrom. The thickness of molten zone 30 is decreased in accord with the relationship

$$l = l_0 - kx \quad (3)$$

where

10  $l$ =the thickness of the molten zone at any time

$l_0$ =the initial thickness of the molten zone

$k$ =the segregation coefficient of the impurity utilized

$x$ =the length of the semiconductor material 29 in crucible 8.

15 The thickness  $l$  of molten zone 30 may be caused to be progressively decreased as a crystal is grown therefrom by any one of several simple expedients. Thus, for example, the thickness may be decreased by causing induction coil 27 to progressively lag farther and farther behind in its downward progress along with the decreasing height of semiconductor material 29 in crucible 8. This may be accomplished by progressively decreasing the pitch of the threads along drive shaft 25 so that coil control mechanism 26 is lowered at a 20 progressively decreasing rate. Alternatively, the radio frequency electrical energy supplied to coil 27 through conductor 35 and 36 may be progressively decreased, thus supplying a lesser amount of heat energy to cause the formation of molten zone 30.

25 30 The amount of significant activator impurities which may be added to molten zone 30 in the practice of the invention are not critical. As a practical matter for single crystal growth there is no reason for adding to the molten layer an amount of impurity which will result in a concentration therein greater than the quantity

$$\frac{S_m}{K} \quad (4)$$

where

40  $S_m$  is the maximum solubility of the activator impurity in the solid semiconductor, and  $K$  is the segregation coefficient of the impurity in the semiconductor.

45 This amount results in the presence, within the growing semiconductor crystal, of the maximum amount of material soluble therein. The addition of an amount of activator impurity to the molten zone which results in a higher concentration therein does not result in the incorporation of a greater amount or concentration of activator impurity within the growing semiconductor crystal. In fact, as greater amounts of activator impurities are added to the molten zone, it eventually becomes difficult to grow single crystals of semiconductor materials therefrom.

50 55 There is, however, no minimum amount which acts as a limit to the amount of activator impurity which may be added to molten zone 30 in the practice of the invention. The addition of the smallest measurable trace of activator impurity to molten zone 30 results in a small but nevertheless detectable amount of activator impurity being deposited in the growing crystal. This may be readily appreciated when it is realized that, in semiconductors such as germanium and silicon, the addition of traces of electrically significant activator impurities as

60 65 small as one part per million has a decided effect upon the electrical characteristics of the semiconductor crystal.

It is, in fact, even possible to practice the invention without adding any significant activator impurity to molten zone 30 through closure 6 prior to growing a crystal therefrom. This may be done by the alternative of using in the case of impurities having a segregation coefficient from 0.5 to 1.0 as a starting material, germanium or silicon having a preselected concentration of electrically significant activator impurities therein. The operation, in this case, results in a uniform distribution in

all but the first and last grown parts of the single crystalline semiconductor ingot of a concentration of activator impurities equivalent to the concentration of the activator impurities in the starting material added to crucible 8. In this case, the first portion of the ingot grown has a concentration of activator impurities less than the concentration of activator impurities within the charge material 29. However, as the crystal is grown, the concentration of activator impurities within molten zone 30 rapidly increases, due to the rejection of the impurity by the growing crystal at a rate inversely proportional to the segregation coefficient of the impurity in the semiconductor. When, however, the concentration of activator impurity within molten zone 30 rises to the value of  $C_s/K$  where  $C_s$  is the concentration of the impurity in the starting material and  $K$  is the segregation coefficient of the activator material in the semiconductor, the concentration of the activator impurity in the remainder of the grown ingot is substantially constant and is equivalent to the concentration of the activator impurity in the starting material. As a practical matter, the first grown portion of the ingot which exhibits a lesser concentration than that of the starting material is a very small portion of the ingot amounting at most to two zone widths, and may readily be detected and discarded.

In the case of impurities in germanium and silicon having a segregation coefficient less than 0.5 and preferably less than 0.01, single crystalline ingots having a substantially constant concentration of impurities therein may be grown without inoculation of the molten zone by an added step of directional cooling of the initial molten mass of semiconductor 29 before the molten zone is formed. Thus, after the initial charge of germanium in crucible 8 has been melted and induction heating coil 27 is adjacent the upper portion of the molten semiconductor within the crucible, the power to induction heating coils 27 and 28 is reduced gradually rather than abruptly so that the semiconductor material 29 within crucible 8 freezes directionally from the bottom of the crucible to the top thereof at a rate of from 5 to 10 inches per hour. This slow directional freezing causes the impurities present within the molten semiconductor to be rejected from the directionally freezing material within the crucible, and causes a concentration of the rejected impurity in the last-frozen portion of the semiconductor within the crucible. Since this last-frozen portion is at the top of the crucible, when the power to induction heating coils 27 and 28 is again increased to form a molten zone at the top of the crucible this molten zone already contains a high concentration of activator impurities and a single crystalline ingot having a substantially constant concentration of impurities therein may be grown therefrom without a further inoculation of the molten zone.

Accordingly, it is evident that the invention may be practiced in two alternative methods. In one method, substantially intrinsic, highly purified semiconductor material is used as a starting material and a preselected activator impurity is added to the molten zone. The concentration of activator impurity which is deposited in the growing zone of crystalline ingot is equal to  $C/K$ . In the other alternative method, the starting material utilized already contains a concentration of one or more activator materials and no addition is made to the molten zone. In this case, the greater portion of the single crystalline ingot grown in accord with the method has a concentration of activator impurities substantially equal to that of the concentration of activator materials in the starting material.

While the broad concept of the practice of the invention has been set forth hereinbefore, the following specific examples are given to illustrate the exact procedure which may be followed in the growing of certain semiconductor crystals having specific constant concentrations of designated impurities therein. These examples are

given for illustrative purposes only and are not to be construed in a limiting sense.

*Example 1.*—The structure illustrated in the drawing is used. In this structure, furnace envelope 1 has a diameter of 4 inches and is 18 inches long. Crucible 8 has an inside diameter of approximately 1 1/4 inches and is approximately 3 inches long. The system is first opened and a seed crystal of single crystalline germanium is inserted in the chuck. Crucible 8 is filled with 300 grams of zone melted germanium having a resistivity in excess of 40 ohm centimeters. The system is then closed and flushed with argon gas at a pressure of 1 atmosphere for approximately 5 minutes. Power is then supplied to induction heating coils 27 and 28 with induction heating coil 27 located adjacent the bottom of crucible 8. A molten zone is formed at the bottom of crucible 8 and the heater is raised manually until the entire charge within the crucible is molten or at a temperature above 941° C. With induction heating coil 27 adjacent the upper surface of the material in the crucible, the power supplied to the coils is slowly reduced until the material in the crucible solidifies and falls to a temperature of approximately 650° C. Power to the induction heating coil is again increased, causing the formation of a molten zone at the top of the solidified germanium in the crucible. Power is adjusted to cause the molten zone to have a thickness of approximately 5/8 inch, and maintained at that level. Ball check valve 7 is then removed from closure 6 and 330 milligrams of antimony are inserted into molten zone 30. Mandrel 18 is then manually lowered until contact is made between the molten zone of germanium and the seed crystal. The seed crystal is maintained in this position until the crystal is observed to begin to melt. Mandrel 18 and drive shaft 25 are then placed on automatic feed by operating suitable clutches in gear box 23, and the seed crystal is rotated at a speed of approximately 100 r.p.m. and withdrawn at a rate of 4 inches per hour. Coils 27 and 28 and molten zone 30 are lowered as the seed crystal is withdrawn at a rate of 2 1/4 inches per hour. At the end of 50 minutes a grown crystal 3 1/2 inches long is withdrawn from the melt leaving the residue of approximately 70 grams of unused germanium at the bottom of the crucible. This crystal is then removed from the chuck and is found to have a resistivity of approximately 0.01 ohm centimeter throughout its length.

*Example 2.*—A single crystal of germanium having therein a substantially constant concentration of arsenic and having a resistivity of approximately 0.01 ohm centimeter is formed using the same procedure as utilized in Example 1 with the addition of 16 milligrams of arsenic to the molten zone instead of the antimony added in Example 1.

*Example 3.*—A single crystal of germanium having therein a substantially constant concentration of phosphorus along its length and having a resistivity of approximately 0.2 ohm centimeter is formed using the procedure described in Example 1 but adding to the molten zone 1.0 milligram of phosphorus instead of the antimony addition of Example 1.

*Example 4.*—A single crystal of germanium having therein a substantially constant concentration of indium and having a resistivity of approximately 1 ohm centimeter is formed using the procedure set forth in Example 1 but adding to the molten zone 2.5 milligrams of indium instead of the antimony of Example 1.

*Example 5.*—A single crystal ingot of germanium having therein a constant concentration of aluminum and having a resistivity of approximately 0.1 ohm centimeter is formed using the procedure of Example 1 but adding to the molten layer 5 milligrams of aluminum instead of the antimony added in Example 1.

*Example 6.*—A single crystal of germanium having therein a constant concentration of gallium and a resistivity of approximately 4 ohm centimeters is formed using

the procedure of Example 1 but adding to the molten zone 7.0 milligrams of gallium.

*Example 7.*—The structure illustrated in Figure 1 of the drawing is used. The dimensions of the structure are the same as those set forth in Example 1. The system is first opened and a seed crystal of single crystal silicon is inserted in the chuck. Crucible 8 is then filled with 150 grams of zone melted silicon having a resistivity in excess of 100 ohm centimeters. The system is then closed and flushed with argon gas at a pressure of 1 atmosphere for approximately 5 minutes. After this period the argon is continually fed into the system to maintain a protective atmosphere. Power is next supplied to induction heating coils 27 and 28 with induction heating coil 27 located adjacent the bottom of crucible 8. A molten zone is formed at the bottom of crucible 8, and the heater is raised manually until the entire charge within the crucible is molten, and at a temperature in excess of 1420° C. With induction heating coil 27 adjacent the upper surface of the material in the crucible, the power supplied to the coils is slowly reduced until the material in the crucible solidifies and falls to a temperature of approximately 1000° C. Power to the induction heating coil is again increased until a molten zone forms at the top of the solidified material within crucible 8. The power is increased until the molten zone has a thickness of approximately  $\frac{5}{8}$  inch. Ball check valve 7 is then removed from closure 6 and 1.2 milligrams of antimony are inserted into molten zone 30. Mandrel 18 is then manually lowered until contact is made between the seed crystal of silicon and the molten silicon. The seed crystal is maintained in this position until the crystal is observed to begin to melt. Mandrel 18 and drive shaft 25 are then connected to automatic feed through gear box 23 and the seed crystal is rotated and withdrawn at a rotation rate of approximately 100 revolutions per minute and a rate of withdrawal of approximately 4 inches per hour. Molten zone 30 progressively falls and induction heating coil 27 is automatically lowered at a rate of  $2\frac{1}{4}$  inches per hour by drive-shaft 25. At the end of 50 minutes the grown crystal approximately  $3\frac{1}{2}$  inches in length and  $\frac{3}{4}$  inch in diameter is withdrawn from the melt, leaving the residue of approximately 35 grams of unused silicon at the bottom of the crucible. This crystal is then removed from the chuck and is found to have a resistivity of approximately 2 ohm centimeters.

*Example 8.*—A single crystal of silicon having therein a substantially constant concentration of aluminum and having a resistivity of approximately 1 ohm centimeter is formed using the same procedure as is utilized in Example 7 with the addition of 1.4 milligrams of aluminum to the molten zone of silicon instead of the antimony addition of Example 7.

*Example 9.*—A single crystal of silicon having therein a substantially constant concentration of gallium along its length and having a resistivity of approximately 0.1 ohm centimeter is formed using the procedure described in Example 7 but adding to the molten zone of silicon 8 milligrams of gallium instead of the antimony addition of Example 7.

*Example 10.*—A single crystal of silicon having therein a substantially constant concentration of indium and having a resistivity of approximately 4 ohm centimeters is formed using the procedure set forth in Example 7 but adding to the molten zone of silicon approximately 8 milligrams of indium instead of the antimony added in Example 7.

Semiconductor single crystals of silicon or germanium impregnated with the hereinbefore described acceptor elements or donor elements produced in accord with the invention have utility as sources of semiconductive materials for the production of semiconductor devices such as rectifiers or transistors. Thus, for example, an ingot of germanium or silicon produced in accord with the invention and having a substantially uniform concentration

of a particular activator impurity therein may be cut transversely into thin slabs approximately 0.05 inch thick which thin slabs may then be cut into square or rectangular wafers which may be used in the production of rectifiers and transistors of the fused junction type as disclosed and claimed in copending application Serial No. 187,478 filed September 29, 1950, now abandoned, and assigned to the same assignee as the present application.

In addition to the formation of semiconductor single crystals having therein a substantially uniform distribution of a single activator impurity, as is described hereinbefore, it is obvious that semiconductor crystals may be formed having therein a substantially uniform concentration of two or more activator impurities. This is due to the fact that the segregation coefficients and the solubilities of electrically significant activator impurities in germanium and silicon are independent of the presence of other impurities therein. Thus, in the practice of the invention, one may add to the constant volume molten zone within the crucible, a quantity of two or more activator impurities, and the process carried on in substantially identical manner, with the production of germanium or silicon ingots having therein substantially constant concentration of two or more activator impurities. Such ingots may then be cut into rectangular cross-sectioned needles or rods of germanium or silicon and used as a starting material for the production of rectifiers and transistors in accord with the local fusion technique described and claimed in copending application of Robert N. Hall, Serial No. 516,637, filed June 20, 1955, now U.S. Patent 2,822,309, and assigned to the same assignee as the present application.

While the invention has been described with respect to certain practices thereof, it will be appreciated that many variations and changes will immediately occur to those skilled in the art. Accordingly, I intend by the appended claims to cover all such modifications that fall within the true spirit and scope of the foregoing disclosure.

What I claim as new and desire to secure by Letters Patent of the United States is:

1. The method of growing unconstrained single crystals of a semiconductor material selected from the group consisting of germanium and silicon having a substantially constant concentration of electrically significant activator impurities therein which method comprises placing a quantity of the semiconductor material in a vertical crucible the depth of which is greater than its diameter, raising the temperature of the semiconductor above its fusion point to cause it to become molten, lowering the temperature of the semiconductor to a temperature below its fusion point but above the temperature at which the semiconductor remains plastic to cause the semiconductor to freeze into a solid but plastic mass, raising the temperature of a zone of the frozen semiconductor mass adjacent to and bounded by the upper surface thereof above the fusion temperature of the semiconductor while maintaining the remainder of the mass at a temperature below the fusion point thereof but above the temperature at which the semiconductor remains plastic to establish a molten zone adjacent the upper surface thereof, contacting the surface of the molten zone with a seed crystal of the semiconductor, and growing a single crystalline ingot of semiconductor by seed crystal withdrawal from the molten zone while replenishing the molten zone from the unmelted portion of said semiconductor mass to maintain the molten zone at a substantially constant volume.

2. The method of growing unconstrained single crystals of a semiconductor material selected from the group consisting of germanium and silicon having a substantially constant concentration of an electrically significant activator impurity therein which method comprises placing a quantity of the semiconductor material in a vertical crucible the depth of which is greater than its diameter,

raising the temperature of the semiconductor above its fusion point to cause it to become molten, lowering the temperature of the semiconductor to a temperature below its fusion point but above the temperature at which the semiconductor remains plastic to cause the semiconductor to freeze into a solid but plastic mass, raising the temperature of a zone of semiconductor adjacent to and bounded by the upper surface of the frozen mass while maintaining the remainder of the mass at a temperature below the fusion point thereof but above the temperature at which the semiconductor remains plastic to cause the creation of a molten zone of semiconductor which comprises only a portion of the total mass of semiconductor within the crucible, contacting the surface of the molten zone with a seed crystal of the semiconductor, and growing a single crystal of semiconductor from the molten zone by seed crystal withdrawal therefrom while progressively melting the remaining solid mass of semiconductor in the crucible to replace the semiconductor removed from the molten zone by growth of the crystal therefrom and maintaining the molten zone at a substantially constant volume.

3. The method of growing unconstrained single crystals of a semiconductor material selected from the group consisting of germanium and silicon having a substantially constant concentration of an electrically significant activator impurity therein which method comprises placing a quantity of the semiconductor material in a vertical crucible the depth of which is greater than its diameter, raising the temperature of the semiconductor above its fusion point to cause it to become molten, lowering the temperature of the semiconductor to a temperature below its fusion point but above the temperature at which the semiconductor remains plastic to cause the semiconductor to freeze into a solid but plastic mass, raising the temperature of a zone of the frozen mass of the semiconductor adjacent to and bounded by the upper surface thereof while maintaining the remainder of the mass at a temperature below the fusion point thereof but above the temperature at which the semiconductor remains plastic to cause the creation of a molten zone of semiconductor adjacent to and bounded by the upper surface thereof which comprises only a portion of the semiconductor in the crucible, and to establish a liquid-solid interface between the lower surface of the molten zone and the unmelted mass of semiconductor remaining in the crucible, contacting the upper surface of the molten zone with a seed crystal of the semiconductor, and growing a single crystalline ingot of semiconductor material by seed crystal withdrawal from the molten zone while progressively lowering the interface between the molten zone and the remaining unmelted semiconductor material to replenish the molten zone with a quantity of semiconductor substantially equal in volume to the amount lost by the growth of the single crystal therefrom and maintain the molten zone at a substantially constant volume.

4. The method of growing unconstrained single crystals of a semiconductor material selected from the group consisting of germanium and silicon and having a substantially constant concentration of electrically significant activator impurities therein which method comprises placing a quantity of the semiconductor material in a vertical crucible the depth of which is greater than its diameter, the semiconductor having a concentration of activator material therein equal to the concentration of activator material desired in the grown single crystal, raising the temperature of the semiconductor above its fusion point to cause it to become molten, rapidly lowering the temperature of the semiconductor to a temperature below its fusion point but above temperature at which the semiconductor remains plastic to cause the semiconductor to freeze non-directionally into a solid but plastic mass, raising the temperature of a zone of the frozen semiconductor mass adjacent to and bounded by the upper surface thereof above the fusion temperature thereof while maintaining the remainder of the frozen mass at a tem-

perature below its fusion point but above the temperature at which the semiconductor remains plastic to establish a molten zone adjacent the upper surface thereof, contacting the surface of the molten zone with a seed crystal of the semiconductor, and growing a single crystalline ingot of semiconductor by seed crystal withdrawal from the molten zone while replenishing the molten zone from the unmelted portion of the semiconductor mass to maintain the molten zone at a substantially constant volume.

5. The method of growing unconstrained single crystals of semiconductor materials selected from the group consisting of germanium and silicon and having a substantially constant concentration of electrically significant activator impurities therein which method comprises placing a quantity of the semiconductor material in a vertical crucible the depth of which is greater than its diameter, raising the temperature of the semiconductor above its fusion point to cause it to become molten, lowering the temperature of the semiconductor to a temperature below its fusion point but above the temperature at which the semiconductor remains plastic to cause the semiconductor to freeze into a solid but plastic mass, establishing a molten zone of semiconductor adjacent to and bounded by the upper surface of the frozen mass of semiconductor while maintaining the remainder of the semiconductor in a solid but plastic state, adding to the molten zone a preselected quantity of an electrically significant activator impurity for the semiconductor having a segregation coefficient in the semiconductor less than unity, contacting the surface of the molten zone with a seed crystal of the semiconductor, and growing a single crystalline ingot of semiconductor by seed crystal withdrawal from the molten zone while maintaining the molten zone at constant volume by replenishment from the solid mass of semiconductor within the crucible.

6. The method of growing unconstrained single crystals of a semiconductor material selected from the group consisting of germanium and silicon having a substantially constant concentration of an electrically significant activator impurity having a segregation coefficient in the semiconductor less than unity therein which method comprises, placing a quantity of the semiconductor material in a vertical crucible, the depth of which is greater than its diameter, the semiconductor having a concentration of activator materials therein equal to the concentration of activator material desired in the grown single crystal; raising the temperature of the semiconductor above its fusion point to cause it to become molten; slowly lowering the temperature of the semiconductor to directionally cool the semiconductor within the crucible from the bottom thereof to concentrate the activator impurities contained therein in the last frozen portion of the semiconductor melt adjacent the upper surface thereof; maintaining the frozen semiconductor mass at a temperature below its fusion point, but above the temperature at which the semiconductor remains plastic; raising the temperature of a zone of the frozen semiconductor mass adjacent to and bonded by the upper surface thereof above the fusion temperature thereof while maintaining the remainder of the frozen mass at a temperature below its fusion point but above the temperature at which the semiconductor remains plastic to establish a molten zone adjacent the upper surface thereof; contacting the surface of the molten zone with a seed crystal of the semiconductor; and growing a single crystalline ingot of semiconductor by seed crystal withdrawal from the molten zone while replenishing the molten zone from the unmelted portion of the semiconductor mass to maintain the molten zone at a substantially constant volume.

7. The method of growing unconstrained single crystals of silicon having a substantially constant concentration of electrically significant activator impurities therein selected from the group consisting of arsenic and phosphorus which method comprises, placing a quantity of the semiconductor material in a vertical crucible the depth

of which is greater than its diameter; raising the temperature of the semiconductor above its fusion point to cause it to become molten; lowering the temperature of the semiconductor to a temperature below its fusion point but above the temperature at which the semiconductor remains plastic to cause the semiconductor to freeze into a solid plastic mass; establishing a molten zone of semiconductor adjacent to and bonded by the upper surface of the frozen mass of the semiconductor while maintaining the remainder of the semiconductor mass in a solid but plastic state; adding to the molten zone a preselected quantity of the chosen electrically significant activator impurity; contacting the surface of the molten zone with a seed crystal of the semiconductor; growing a single crystalline ingot of the semiconductor by seed crystal withdrawal from the molten zone; continuously replenishing the molten zone from the solid mass of semiconductor within the crucible at a rate which continuously decreases the thickness of the molten zone so that the thickness of

5

10

15

the molten zone at any time is defined by the relationship  $l = l_0 - kx$  where

$l$ =the thickness of the molten zone at any time

$l_0$ =the initial thickness of the molten zone

$k$ =the segregation coefficient of the impurity utilized

$x$ =the length of the semiconductor material remaining in the crucible at the given time

References Cited in the file of this patent

UNITED STATES PATENTS

|           |               |               |
|-----------|---------------|---------------|
| 2,631,356 | Sparks et al. | Mar. 17, 1953 |
| 2,727,840 | Teal          | Dec. 20, 1955 |
| 2,739,088 | Pfann         | Mar. 20, 1956 |
| 2,747,971 | Hein          | Mar. 29, 1956 |

OTHER REFERENCES

Bell Tel. Lab. Inc. and Western Electric Inc., "Transistor Technology," July 1952, Parts I and II.